

10/6  
10/94  
Patented Oct. 17, 1922.

1,432,545

## UNITED STATES PATENT OFFICE.

LAURENCE J. GILBERT, OF VICKSBURG, MISSISSIPPI.

## INVESTMENT MATERIAL.

No Drawing.

Application filed August 3, 1921. Serial No. 489,620.

*To all whom it may concern:*

Be it known that I, LAURENCE J. GILBERT, a citizen of the United States, and resident of Vicksburg, in the county of Warren and State of Mississippi, have invented a certain new and useful Improvement in Investment Materials, of which the following is a full, clear, concise, and exact description.

My invention relates to an investment material suitable for use by dentists in making all sorts of cast and soldered dental restorations.

All of the ingredients of my improved investment are comparatively cheap, and the investment material is made from these ingredients by simple, mechanical mixture in the proportions hereinafter set forth.

The investment material of my invention is capable of setting and drying quickly, will not expand, contract, or break under heating, and, even under high temperatures, will not in any way mar or discolor porcelain or other white teeth with which the investment may be in contact.

My investment material economizes time for the dentist, as it can be placed over a gas or other flame five to ten minutes after mixing, and dries out quickly.

My investment material is particularly useful in making soldered bridges, because the investment will not mar or discolor white teeth, as before stated, and by reason of the further fact that the investment is capable of visually indicating to the operator when the investment and the bridge parts supported therein have been heated to the temperature at which gold solder should be flowed over the several bridge parts to secure the same together.

Having thus made a preliminary statement of the purposes, objects, and advantages of my invention, I shall now describe the investment in detail. The ingredients of my improved investment are silica, Portland cement, and (dental) plaster of Paris, mechanically mixed together in the following proportions (by measure) to wit:—

Silica----- 2 parts.  
Portland cement----- 3 parts.  
(Dental) plaster of Paris----- 1 part.

Each of the ingredients is preferably in finely divided or powdered form, prior to the measurement thereof. The completed in-

vestment material resulting from the mixture of said ingredients is dark gray in color. Immediately prior to use the dark gray investment material is mixed with sufficient water to give the mixture substantially the consistency of bread dough.

It will be unnecessary to explain how the investment material is used in making inlays, onlays, dummies, plates and other cast restorations, since all persons familiar with prosthetic dentistry will understand how to use the investment material for such purposes. It will suffice to state that my investment is especially adapted for use in dental casting, because it sets and dries very quickly, because it will not expand, contract, or break under heating, and because after the completion of the casting operation the investment may be easily and cleanly broken away from the finished casting.

The color changing characteristic of my investment is also advantageous in dental casting, because the change in color advises the operator that his investment is hard and dry, that his pattern has burned out, (if he uses a wax pattern) and that his investment mold has been heated to the temperature which should be obtained before he forces his gold (or other metal) into the cavity of the mold.

Bridges are ordinarily made by soldering porcelain teeth (or gold dummies) to an abutment or abutments, the abutments being in the form of crowns or inlays. Prior to soldering the several parts of the bridge together, the same are positioned upon a plaster or other model of the patient's mouth. The bridge parts are then invested, the back (lingual surfaces) thereof being left exposed. The invested case is then gradually heated to the melting point of eighteen carat gold solder, and then with the aid of a hydrogen or other suitable blow pipe the solder is flowed over the abutments and intermediate teeth to secure the same together.

My improved investment is especially useful in constructing bridges by the method mentioned in the preceding paragraph, because it will not expand, contract, or break under heating, and because it will not mar or discolor the porcelain teeth. As stated before, the investment is dark gray in color. Under heating, the investment material changes color and finally becomes as white

as chalk when it has been heated to the melting point of eighteen carat gold solder. Thus, the operator knows that when his investment has become white it is time for 5 him to flow his solder.

Having thus described the investment material of my invention, what I claim as new and desire to secure by Letters Patent of the United States is:

- 10 1. A dental investment material consisting of a major portion of Portland cement, and minor portions of silica and plaster of Paris.
- 15 2. A dental investment material consisting of plaster of Paris, and relatively greater portions of silica and Portland cement.
- 20 3. A dental investment material consisting of silica, Portland cement and plaster of Paris, the Portland cement being present in greater quantity than either of the other

ingredients and the silica being present in greater quantity than the plaster of Paris.

4. A dental investment material which comprises silica, Portland cement and plaster of Paris, in the following proportions; (by measure) to-wit;

|                  |       |            |
|------------------|-------|------------|
| Silica           | ----- | 2 parts.   |
| Portland cement  | ----- | 3 parts.   |
| Plaster of Paris | ----- | 1 part. 30 |

5. A dental investment material which consists of Portland cement, and quantities of silica and plaster of Paris, which together measure substantially equal to the Portland cement. 35

In witness whereof, I hereunto subscribe my name this 14th day of July, 1921.

LAURENCE J. GILBERT.

Witnesses:

JUD G. GREENWAY,  
HARRY YOSTE.